

J. F. MONNOT,  
PROCESS OF MAKING CLAD METAL ARTICLES,  
APPLICATION FILED JUNE 13, 1908.

927,371.

Patented July 6, 1909.

Fig. 1.



Fig. 2.



Fig. 3.



Attest:

W. D. Nichols  
A. M. Doughton

by

Inventor:  
John F. Monnot,  
Marble & McElroy  
Atty's

# UNITED STATES PATENT OFFICE.

JOHN F. MONNOT, OF NEW YORK, N. Y., ASSIGNOR TO DUPLEX METALS COMPANY, OF NEW YORK, N. Y., A CORPORATION OF NEW YORK.

## PROCESS OF MAKING CLAD-METAL ARTICLES.

No. 927,371.

Specification of Letters Patent.

Patented July 6, 1909.

Application filed June 13, 1908. Serial No. 438,396.

*To all whom it may concern:*

Be it known that I, JOHN F. MONNOT, a citizen of the United States, residing at New York, in the county of New York and State 5 of New York, have invented a certain new and useful Process of Making Clad-Metal Articles; and I do hereby declare the following to be a full, clear, and exact description of the same, such as will enable others skilled 10 in the art to which it appertains to make and use the same.

My invention relates to a process of making clad metals; by which term is meant bodies comprising a core or base of one metal 15 (iron or steel for instance) having united thereto, and preferably inseparably united or welded thereto, a substantial layer or coating of metal, usually an unlike metal, (for instance, copper, silver, gold, aluminum, 20 brass, bronze, aluminum bronze, etc.). In particular, my invention comprises a process of making clad metal ingots; which ingots, when formed, may be rolled, pressed, hammered, or otherwise extended down to rods, 25 sheets, bars, strips, wire and other commercial or desired forms.

In various prior patents and applications for patents, for example, Patents Nos. 851,993, 853,716, and applications Sr. Nos. 30 281,680, 391,673, and 400,843, I have illustrated and described processes and apparatus for producing clad metal bodies or ingots such as referred to, and comprising various pairs of unlike metals such as referred 35 to inseparably welded together, such processes being based on a discovery made by me, to the effect that various metals, copper and silver for example, which do not form a permanent or weld-like union with iron or steel 40 when cast against an iron or steel surface at ordinary casting temperatures, do form permanent weld-like unions when raised to a much higher temperature (termed by me, for the sake of a name, the "supermolten" 45 temperature,) and contacted with the iron or steel surface. The said patents and applications disclose methods of and means for contacting a solid base of one metal, steel for example, with molten metal of an unlike 50 nature, copper for example, under such conditions of temperature and physical contact that union will take place.

A process involving the casting of the core or base metal, which is usually relatively 55 large in amount inside of or against the sur-

face of the metal which is to form the covering or coating of the ingot or other article to be produced and which is usually relatively small in amount—for example, a process involving the casting of a steel core or 60 base inside of a copper shell—has numerous advantages from a practical point of view. In such a process, ingots of any desired size may be produced; the apparatus required is proportionately less expensive and more 65 easily handled, little manipulation is necessary, it is not necessary to employ crucibles of great size for containing molten coating metal and to take extreme care during manipulation to avoid oxidation of the coating 70 metal or of the surface of the core to be coated; and numerous other advantages might be pointed out. The practical impossibility of casting steel or like cores or bases in such manner as to avoid pores, 75 bubbles, blow-holes, pipes, and the like, and the great difficulty of preventing oxidation of the surface of the copper or other coating during the casting but prior to the actual covering of the surface with the molten 80 metal and of preventing oxidation of the surface of the cast metal, as well as other difficulties which might be mentioned, have militated against the use of any such process, however. To produce a metallic union 85 between two metals it is necessary that such metals shall come into contact with clean, truly metallic surfaces, free of infusible oxids or impurities, along the line of intended union. It has been difficult, furthermore, to prevent the cast steel core from pulling away from the solid coating, during the solidification and shrinking of the cast core. And in uniting a molten high-melting 90 core metal with a solid lower-melting coating metal, there has been extreme probability that the coating metal will be contaminated to a considerable extent by the core or base metal, owing to partial fusion of the coating metal and consequent mingling of the two 100 metals. Such contamination is exceedingly objectionable in many cases; for example, in the making of metal for electrical conductors.

The method of casting metal ingots set 105 forth in my application Sr. No. 391,674, involving the passing of the molten metal through a layer of molten "wiping material", such as a suitable flux, and the retarded cooling of a large body of molten metal at 110

the top of the ingot, so that this body will remain fluid after the main portion of the ingot has set and will flow down to fill any "pipes" or the like which may form, and 5 will also exert a certain amount of fluid pressure to solidify the metal, overcomes these difficulties, and makes it possible to cast a steel core inside of a copper shell, and to obtain a dense, solid core; and the same 10 layer of "wiping material" through which the metal for this core is cast, also serves to remove any layer of oxid or other contamination on the surface of the said shell, besides preventing contact of the air with the portion of the solid metal immediately above 15 the molten metal and necessarily heated to a high temperature. This layer of "wiping material" further removes entrained and occluded gases, oxid impurities, etc. from 20 the molten metal, preventing the formation of bubbles, blow-holes or blebs where the cast metal core contacts with the said coating metal and allowing a full-area contact between truly metallic surfaces of the two 25 metals. It is extremely important, in the making of clad metal articles intended to be extended or worked, to avoid any such flaws at the surface of union, as any such flaws, if formed, extend greatly during the subsequent 30 working and extension of the clad metal, producing what may prove to be serious defects in the final product. For example, in the case of clad metal ship plates, consisting of a steel base or back and a copper, brass, bronze, Tobin bronze, or like 35 coating, a bubble or blow-hole at the line of union in the large ingot, may in the final plate form a lineal flaw or pore which will admit sea-water to the steel back, permitting 40 galvanic action between the metals of the back and of the coating, which will result in the weakening and finally in the perforation of the plate. Casting the molten steel through "wiping material", as described, 45 avoids the presence of the gas to which such bubbles or blow-holes are due, permitting the two metals to come into absolute metallic contact at all meeting points. This method of casting through molten "wiping material" also makes possible the casting 50 of the metal of the said shell or coating itself, immediately in advance of the casting of the metal of the core or base. Heretofore this has not been practicable, because cast copper or like metal usually contains numerous 55 internal flaws, blow-holes, etc., which make it necessary to roll or otherwise work it before it can be used as such a coating or shell. But metal cast through "wiping material" is practically free from such internal 60 flaws.

The preferred method of carrying out my present process, therefore, supposing the article to be produced to be an ingot composed 65 of a steel core and a copper or other non-fer-

rous coating, comprises casting the metal for this coating in a suitable mold containing a collapsible or otherwise removable core adapted to form inside the coating a space sufficient for the cast core, such casting being 70 done through a layer of molten "wiping material"; in removing the said collapsible core as soon as the metal for said coating has set, and in then casting into the space from which such core was removed, the molten steel to 75 form the core of the ingot, such casting being also done through a layer of molten "wiping material". And preferably, to cause rapid shrinking of the coating, so that there can be no separation of the cast core from it, I chill 80 the mold as soon as, or soon after, the core has been cast. This chilling is further advantageous in many cases, because copper and many other metals are softer, closer-grained, and altogether better if cooled 85 quickly from the molten state. This chilling also obviates fusion of the coating metal and consequent mingling of the two metals, with consequent impairment of quality of the 90 metal of the coating.

In the accompanying drawing I illustrate apparatus for carrying out my said process, and the manner of carrying it out.

Figure 1 shows a central vertical section of one form of mold which may be used, and with 95 one form of collapsible core which may be used in place in said mold; also a layer of molten metal for the coating, in the annular space between the core and sides of the mold, and a layer of molten "wiping material" above 100 such molten metal. Fig. 2 shows a similar section (except that the section is not taken through the two "runners", as is the section of Fig. 1) of the mold after the shell for the coating has been cast and solidified, and after 105 the collapsible core has been removed and the runner for pouring the metal for the ingot core has been put in place. Fig. 3 shows a horizontal section of the mold and collapsible core, on the line x-x of Fig. 1.

In the drawings, 1 designates an ingot mold, which in most cases may be of iron; and 2 designates a collapsible core of the size required to give the desired size of cast core in the final ingot.

3, 3, designate inclined runners on opposite sides of the mold, through which molten metal for the coating may be poured into the mold from two sides at once.

4 designates a cooling jacket with which 120 the mold may be provided, and which is provided with means for introducing into it or circulating through it any suitable cooling fluid, such as water, oil, brine, air, etc.; and air or other suitable gas under pressure may 125 be expanded in this jacket to produce the desired cooling.

The collapsible core 2 may be of any suitable construction. I have shown a core comprising a central tapered wedge 5 of rectan- 130

5 gular section, provided at its upper end with a ring-bolt 6 by which it may be lifted, and four side-pieces 7. The mold 1 has at its bottom a shallow recess 8 in which the lower end of the core may be stepped, said recess serving to center the core and also to hold its sections together at the bottom; and at its upper end the core has a clamp 9 which serves to hold its sections together.

10 Fig. 2, designates a runner of refractory material which is applied to the mold after the shell for the coating has been cast and when the metal for the ingot core is to be cast.

15 The mold 1 is preferably formed of a plurality of sections secured together, which purpose I have shown clamping rings 11 and wedges 12. The mold shown is made in two sections, so that it will part to permit removal of the cast ingot. A mold made in a greater number of sections will serve as well, or even better. It is desirable to avoid employing a mold with material draft, so that the coating may be of substantially the 20 same thickness, and the cast core of substantially the same diameter, at the top as at the bottom; and employing a mold which parts longitudinally make it possible to avoid draft in the mold.

25 The method of carrying out the process is as follows: The parts of the mold having been clamped together, as shown in Figs. 1 and 2, and the collapsible core 2 being in place as indicated in Figs. 1 and 3, and the 30 inside of the mold and the surface of the core 2 having preferably been given a coating of a suitable substance, for example a graphite mixture or wash, to prevent the molten metal clinging to them, molten metal, copper for 35 example, is poured into the annular space between the core 2 and the sides of the mold, through a layer 13 of molten wiping material previously introduced, the metal being preferably introduced from a plurality of points 40 simultaneously so that it will fill the mold quickly. In descending through the layer of wiping material, which should be of substantial thickness, the molten metal is freed 45 of adhering, absorbed and entrained moisture and gases so that the several drops or 50 bodies of such metal meet beneath the layer with clean, readily coalescing surfaces, forming a sound and perfect casting. And as the molten wiping material rises above the accumulating molten metal, it similarly wipes the 55 surfaces of mold and core, permitting the casting to take an accurate shape and have a good surface, free of blebs, pitholes, etc. The molten copper is poured in until it about 60 reaches the top of the jacket 4, and then the pouring is stopped, and the molten metal is permitted to solidify. To hasten solidification, cooling water or other cooling fluid may 65 be introduced into or circulated through the jacket 4, though in general cooling will not

be necessary at this point. As soon as the molten metal, which now forms a shell 14, has set, and while it is still red hot or hotter, the collapsible core 2 is removed, the layer of wiping material now flowing down to the bottom of the central space 15 from which the core 2 was removed, the runner 10 is put in place, and molten steel for the core is poured into this central space, through the wiping material, which rises as the steel fills the central space 15. Steel is so poured in until space 15 is full and the runner 10 is also partly filled with the molten metal, the molten wiping material then forming over the top of the molten metal a protective covering of relatively low heat conductivity; and since the runner 10 is also of a material of low heat conductivity, cooling of the molten metal in the runner is relatively slow. As soon as the mold has been filled as described 70 water or other suitable cooling fluid is admitted to or circulated through cooling jacket 4, so preventing the copper shell from melting and chilling the shell and causing it to contract with the cast steel inside it. As the copper shell cools it will in turn cool the adjacent portion of the cast steel core, causing the metal below the runner to cool more rapidly than the metal within the runner, the latter metal remaining liquid until the 75 metal below has fully set. Any pipes or the like which may form during the solidification of the cast core are filled by downflow of metal from the runner; and the fluid pressure exerted by the metal in this runner also helps to insure good density of the cast metal. Preferably the ingot so cast is removed from the mold as soon as practicable and is immediately worked, by rolling or otherwise; or it may be subjected to pressure while still fluid 80 in the mold, according to well-known methods of pressure-casting.

85 The casting of both metals through molten "wiping material" as described removes all 90 oxid, and like impurities, entrained and occluded gases, and insures a particularly good 95 quality of metal, if the process is carried on properly. Oxidation of the metal during the casting is precluded, since the molten metal in the mold is at all times covered by an air-excluding layer of wiping material. Various 100 different wiping materials may be used; one suitable material being a mixture of sodium 105 or potassium silicate, borax and boric acid.

110 Of course my process described above is not limited to the production of the shell 14 by casting as described; the shell 14 may be produced in any suitable manner, and placed solid within the mold, if desired. And it 115 would be an obvious modification of the process above described to cast the steel core within a sectional mold contained within mold 1, remove the said sectional mold when the steel core is solid, and then 120 cast molten coating metal, through wiping 125

material, into the space between said core and the sides of mold 1; afterward working the ingot as described. It may be that the steel, when it first contacts with the solid 5 copper, produces actual or incipient fusion of the copper on the extreme surface; such fusion, if it occurs, facilitating the formation of a union between the two metals. But the cooling of the copper shell as described prevents any material fusion such as will result 10 in material contamination of the copper by the metal of the core.

If desired or required, after the removal of the collapsible core from the mold, after 15 casting the annular body 14, additional flux or wiping material may be poured into the interior of such annular body to completely fill it, so absolutely protecting its surfaces from oxidation and removing any trace of 20 oxid which may have been already formed, so that an absolutely clean surface of the metal is exposed when the molten steel displaces this flux or wiping material.

I do not limit the process to top pouring, 25 but may pour through the bottom of the ingot mold, as is common in steel practice, if desired.

It is obvious that the same process above described is equally applicable to the formation 30 of objects in which neither metal completely surrounds the other; for example, objects in which one body of metal abuts against, without surrounding, the other; in such case the mold used will have a removable 35 filling piece, corresponding to the collapsible core 2, which will fill that portion of the mold which is to be occupied by the body of metal cast last; and the body of metal first cast will be cast into the remaining 40 portion of the mold, and after it has solidified the said filling piece will be removed and the other body of molten metal cast.

Instead of first casting a copper or like metal body, permitting it to solidify, and 45 then casting molten steel against the surface of the solidified copper or other metal, I may cast the steel and the non-ferrous metal practically simultaneously, by placing a suitable separator in the mold and casting the one 50 metal on one side of the separator and the other metal on the other side of the separator; casting both metals through molten wiping material, as already described, so as to obtain dense, sound metal free from blow-holes and the like. Thus, in the making of a 55 copper-steel round ingot, I may place a steel tube of suitable size in the mold, and cast copper, through flux, either inside or outside the tube, according as the copper is desired either on the inside or outside of the finished 60 product, casting the steel on the opposite side of the tube, casting through flux or wiping material in both cases. And in making flat or square ingots the same method may 65 be employed, a suitable separator being

placed in the mold to keep the two metals separate during the pouring. In casting by this method, both metals will weld to the separator, and so will in effect be welded to each other.

The methods of making clad or compound metal ingots of unlike metals, casting the steel against a solid, lower-melting metal, described in this specification, has the important advantage over methods of making such 70 ingots involving the casting of copper or the like on a solid core or base of iron or steel, as described in prior patents issued to me, that the ingot may be rolled, without reheating, immediately after the steel has solidified and 80 while it is still at a much higher temperature than the copper or other coating metal. Rolling clad metal ingots produced by casting the copper or the like about the steel, presents certain practical disadvantages, 85 owing to the fact that the ingot must be rolled at a temperature at which the copper or like metal is solid, which is not necessarily the best working temperature for the particular steel employed; and after the ingot is once 90 produced, it can be heated only from the outside, that is to say, through the copper or like metal, so that on such reheating its interior temperature cannot be higher, initially, than its exterior temperature. But when the ingot, produced as described herein, is rolled without reheating, the steel may be at a much higher temperature than the copper, first because it solidifies at a higher temperature, the copper being kept at a lower temperature 100 in the mold by the cooling means described, and then when the ingot is removed from the mold and rolled, radiation of heat to the air and the higher heat conductivity of the copper will keep the temperature 105 of such copper materially lower than that of the steel inside. For this reason the ingot so produced is much easier to work by rolling or otherwise, and no reheating before rolling is 110 required.

What I claim is:—

1. A process of making clad metal objects which comprises forming a compound ingot by casting molten metal of relatively high melting point through a layer of molten 115 wiping material in an ingot mold and against the surface of a solid body of metal of lower melting point and causing it to solidify thereagainst.

2. A process of making clad metal objects 120 which comprises casting molten metal of relatively high melting point through a layer of molten wiping material against the surface of a solid body of metal of lower melting point and causing it to solidify thereagainst, 125 and abstracting heat from the solid metal during contact with such molten metal.

3. A process of making clad metal objects which comprises forming a compound ingot by casting molten metal of relatively high 130

melting point through a layer of molten wiping material into the interior of an annular body of metal of lower melting point, and causing it to solidify against the surface of such annular body.

4. A process of making clad metal objects which comprises casting molten metal of relatively high melting point through a layer of molten wiping material into the interior 10 of an annular body of metal of lower melting point, causing it to solidify against the surface of such annular body and abstracting heat from such annular body during contact thereof with the molten metal.

15 5. A process of forming clad metal objects which consists in casting a molten body of ferrous metal through a layer of molten wiping material into contact with a solid body of metal consisting in whole or in greater 20 part of non-ferrous metal, and permitting the molten metal to solidify against such body.

6. A process of forming clad metal objects which consists in casting a molten body of ferrous metal through a layer of molten wiping material into contact with a solid body of copper and permitting the molten metal to solidify against such body.

7. A process of forming clad metal objects which consists in casting a molten body of ferrous metal through a layer of molten wiping material into contact with a solid body of metal consisting in whole or in greater part of non-ferrous metal, and permitting the molten metal to solidify against 35 such surface and abstracting heat from such solid metal during contact thereof with the molten metal.

8. A process of forming clad metal objects which consists in casting a molten body of ferrous metal through a layer of molten wiping material into contact with a solid body of copper and permitting the molten metal to solidify against such body and abstracting heat from such solid metal during 45 contact thereof with the molten metal.

9. A process of forming clad metal objects which consists in casting molten ferrous metal through a layer of wiping material into the interior of an annular body of metal 50 consisting in whole or greater part of non-ferrous metal and permitting such molten metal to solidify against such body.

10. A process of forming clad metal objects which consists in casting molten ferrous metal through a layer of wiping material into the interior of an annular body of metal 55 consisting in whole or greater part of copper and permitting such molten metal to solidify against such body.

11. A process of forming clad metal objects which consists in casting molten ferrous metal through a layer of wiping material into the interior of an annular body of metal 60 consisting in whole or greater part of non-ferrous metal and permitting such molten metal to solidify against such body, and

abstracting heat from such annular body during contact thereof with the molten metal.

12. A process of forming clad metal objects which consists in casting molten ferrous metal through a layer of wiping material into the interior of an annular body of copper and permitting such molten metal to solidify against such body, and abstracting heat from such annular body during contact thereof with the molten metal.

13. A process of forming clad metal objects which consists in contacting with the surface of a solid body of metal a layer of molten flux comprising oxid-dissolving material, casting through such layer of flux into contact with the surface of such metal, a body of molten metal of higher melting point and by the progressive rise of the layer of flux removing oxid from the surface of the solid metal and exposing a clean surface of such metal to contact with the molten metal, and permitting the molten metal to solidify against such surface.

14. A process of forming clad metal objects which consists in contacting with the surface of a solid body of metal a layer of molten flux comprising oxid-dissolving material, casting into contact with such surface a body of molten metal and causing the molten metal so cast to raise the layer of flux and thereby to expose progressively a clean surface of the solid metal to contact with the molten metal, and permitting the molten metal to solidify against such surface.

15. A process of forming clad metal objects which consists in contacting with the inner surface of an annular body of metal a layer of molten flux comprising oxid-dissolving material, casting into the space within said annular body a body of molten metal and causing the molten metal so cast to raise the layer of flux and thereby to expose progressively a clean surface of the solid metal to contact with the molten metal, and permitting the molten metal to solidify against such surface.

16. A process of forming clad metal objects which comprises casting a body of molten metal and permitting it to solidify, producing a substantial layer of flux next a surface of the body so formed and while said body is hot casting into contact with its said surface through said layer another body of molten metal and causing such metal to displace said flux, and permitting such second body of molten metal to solidify against such surface.

17. A process of forming clad metal objects which comprises casting a body of molten metal and permitting it to solidify, producing a substantial layer of flux next a surface of the body so formed and while said body is hot casting into contact with its said surface through said layer another body of

- molten metal and causing such metal to dis-  
place said flux, permitting such second body  
of molten metal to solidify against such sur-  
face, and abstracting heat from such first  
body of metal during contact thereof with  
said second body of molten metal.
18. A process of forming clad metal ob-  
jects which comprises casting a body of mol-  
ten metal through a layer of wiping material,  
10 and permitting the metal to solidify, and  
while said body is hot casting into contact  
with a surface of it, through a layer of wiping  
material, another body of molten metal, and  
permitting such second body of molten metal  
15 to solidify against such surface.
19. A process of forming clad metal ob-  
jects which comprises casting a body of mol-  
ten metal through a layer of wiping material,  
20 and permitting the metal to solidify, and  
while said body is hot casting into contact  
with a surface of it, through a layer of wiping  
material, another body of molten metal,  
permitting such second body of molten metal  
25 to solidify against such surface, and abstract-  
ing heat from such first body of metal during  
contact thereof with said second body of  
molten metal.
20. A process of forming clad metal ob-  
jects which comprises casting a body of mol-  
ten metal through a layer of wiping material,  
30 and permitting the metal to solidify, pro-  
tecting a surface of such body from oxida-  
tion with molten flux and while said body is  
hot casting into contact with such surface,  
35 through flux, another body of molten metal,  
and permitting such second body of molten  
metal to solidify against such surface.
21. A process of forming clad metal ob-  
jects which comprises casting a body of mol-  
ten metal and permitting the metal so cast  
to solidify while protecting such metal  
against oxidation, casting into contact with  
the surface of the body so produced another  
body of molten metal under conditions pre-  
cluding oxidation and permitting it to  
solidify against the surface of said first body,  
and abstracting heat from said first body of  
metal at such rate as to permit refusion of  
only a thin layer thereof adjacent the second  
body of metal, thereby insuring molecular  
50 contact of the two metals and avoiding ma-  
terial mixing thereof.
22. A process of working, by rolling, press-  
ing, hammering or the like, clad metal bodies,  
which consists in maintaining the core, of  
55 metal of higher melting point, at a tem-  
perature higher than that of the coating,  
of metal of lower melting point, and working  
same by rolling, pressing, hammering or the  
like while maintaining a temperature differ-  
ential between the two metals.
23. A process of forming compound metal  
objects which comprises placing a separator  
in a suitable mold and casting different kinds  
or grades of metal, through molten wiping  
65 material, on opposite sides of said separator  
causing the two metals in solidifying to weld  
to the separator and so to each other.
- In testimony whereof I affix my signature,  
in the presence of two witnesses.
- JOHN F. MONNOT.

Witnesses:

H. M. MARBLE,  
K. G. LE ARD.